

## UNITED STATES PATENT OFFICE

WILLIAM B. PRICE, OF WATERBURY, CONNECTICUT, ASSIGNOR TO SCOVILL MANUFACTURING COMPANY, OF WATERBURY, CONNECTICUT, A CORPORATION OF CONNECTICUT

## NONFERROUS ALLOY

No Drawing.

Application filed April 16, 1931. Serial No. 530,735.

This invention relates to an improvement in non-ferrous alloys and particularly to an alloy whose principal constituent is copper, this being accompanied in the present invention by zinc, as well as by small but essential proportions of nickel and aluminum. The physical properties of the alloy in its different conditions were found to be as follows:

55

|                  | Soft annealed | Light annealed | Hard    |
|------------------|---------------|----------------|---------|
| Yield point      | 17,000        | 57,000         | 116,000 |
| Tensile strength | 58,000        | 78,000         | 119,000 |
| Elongation       | 58%           | 33%            | 4%      |

66

The alloy was tested for tensile strength, elongation (in 2 inches) and reduction of area, with the following results:

65

| Temperature | Tensile strength<br>lbs. per sq. in. | Elongation per cent | Reduction in area, per cent |
|-------------|--------------------------------------|---------------------|-----------------------------|
| 500°C.      | 16,600                               | 40                  | 49                          |
| 625°C.      | 7,700                                | 49                  | 52                          |
| 750°C.      | 4,200                                | 101                 | 89                          |
| 875°C.      | 2,000                                | 142                 | 100                         |
| 950°C.      | 1,300                                | 128                 | 100                         |

70

The alloy of the present invention has a high resistance to corrosion and oxidation, and retains a relatively high resistance to oxidation at elevated temperatures, there being substantially no change in color or evidence of oxidation at temperatures up to 600°C.

75

It was found that the freedom of the alloy from tin was particularly important in the manufacture of condenser tubes from ingots of the alloy by extrusion methods. When tin was present, even in small amounts, the ingot could not be extruded in a special tube extrusion machine of 900 tons capacity, unless the ingots were heated to a high temperature, for example, above about 950°C., at which the tin liquated. By omitting the tin the alloy could be readily extruded at the customary temperatures and pressures of working.

85

Also by omitting the tin the resistance to corrosion and oxidation at elevated temperatures was greater than when tin was present.

90

Extruded condenser tubes made from the alloy of the present invention gave, when 100

The preferred composition of the new alloy is:

|          | Per cent |
|----------|----------|
| Copper   | 80       |
| Aluminum | 2        |
| Nickel   | 1        |

25

The remainder of the alloy is substantially all zinc, and in no case must there be any appreciable amount of tin present.

In commercial practice an alloy made from commercial material proportioned to give the composition above stated, when analyzed showed the following composition:

|          | Per cent |
|----------|----------|
| Copper   | 80.16    |
| Aluminum | 2.07     |
| Nickel   | 1.00     |
| Zinc     | 16.77    |

The percentage of zinc was determined by difference and of course might include traces of impurities, for example, lead, iron or other ingredients, which, however, if present, were in too small an amount to affect the properties of the alloy.

This commercial alloy when cast in a slab of about  $\frac{3}{4}$  inch thickness had a hardness of 45 Brinell.

The cast slab was rolled to a thickness of 0.151 inches and then annealed for one hour at 750°C. to relieve it of internal stresses,

95

tested, at normal temperatures, the following results:

|                     | Tensile strength<br>lbs. per<br>sq. in. | Yield<br>point lbs.<br>per sq.<br>in. | Elonga-<br>tion per<br>cent in<br>2" |
|---------------------|-----------------------------------------|---------------------------------------|--------------------------------------|
| Hard                | 119,900                                 | 116,000                               | 4                                    |
| Relief annealed     | 78,000                                  | 37,000                                | 33                                   |
| Annealed at 650° C. | 58,000                                  | 17,000                                | 55                                   |

**10** What is claimed is:

1. An alloy comprising essential amounts of copper, aluminum and nickel in proportions substantially within the following ranges:

|          | Per cent |
|----------|----------|
| 15       |          |
| Copper   | 80 to 85 |
| Aluminum | 1 to 2½  |
| Nickel   | 1 to 2½  |

20 2. An alloy consisting of the following ingredients in proportions substantially as stated:

|             | Per cent |
|-------------|----------|
| Copper      | 80       |
| 25 Aluminum | 2        |
| Nickel      | 1        |
| Zinc        | 17       |

In testimony whereof, I have hereunto set my hand.

## 30 WILLIAM B. PRICE.

35

40

48

50

65

60

65